# EUROPEAN PATENT SPECIFICATION

(11) **EP 2 491 167 B1**
(45) Date of publication and mention of the grant of the patent: **10.07.2019**
(21) Application number: 10773461.8
(22) Date of filing: 19.10.2010
(51) Int. Cl.: C25D 5/18, C25D 5/48, C25D 9/08

(54) **METHODS OF DEPOSITING DISCRETE HYDROXYAPATITE REGIONS ON MEDICAL IMPLANTS**
VERFAHREN ZUR AUFTRAGUNG VON EINZELNEN HYDROXYAPATITREGIONEN AUF MEDIZINISCHE IMPLANTATE
PROCÉDÉS DE DÉPÔT DE RÉGIONS INDIVIDUELLES D'HYDROXYAPATITE SUR DES IMPLANTS MÉDICAUX

(30) Priority: 19.10.2009 US 581483
(43) Date of publication of application: 29.08.2012
(73) Proprietor: Biomet Manufacturing, LLC, Warsaw, IN 46582 (US)
(72) Inventor: GUPTA, Gautam, Warsaw Indiana 46582 (US); SEWING, Andreas, 12163 Berlin (DE)
(74) Representative: Manitz Finsterwald Patent- und Rechtsanwaltspartnerschaft mbB
(86) International application number: PCT/US2010/053138
(87) International publication number: WO 2011/049915

(56) References cited:
- WO-A1-98/09006
- WO-A1-98/13539
- WO-A2-2008/146113
- DE-A1- 10 158 302
- US-A- 5 310 464
- US-A1- 2002 084 194
- US-B2- 6 764 769

## Description

### INTRODUCTION

The present technology relates to medical implants having discrete regions of a calcium phosphate (e.g., hydroxyapatite), and methods of their manufacture. In the growing field of medical devices, there is a continued need to provide lightweight orthopedic implants having enhanced in-growth capability. It is known that the time between in-growth of a metallic implant until the full mechanical loadability is achieved can be reduced if the implant has been coated with a calcium phosphate phase (CPP), such as hydroxyapatite.

Hydroxyapatite is a biocompatible material similar in composition to the mineral content of natural bone. As a result, hydroxyapatite coatings on medical orthopedic implants can enhance the implant's osteoconductive potential, among other things. CPP coatings can be deposited onto electroconductive, or metal substrates using solution-based techniques, such as electrochemical deposition or sol-gel deposition. One advantage of using such deposition processes is that they are not "line of sight" processes and thus can provide a complete coating coverage of complex shaped substrates. With the use of implants having nano-scale texturing, however, such deposition processes can be disadvantageous in that the coating may be applied over the nano-scale texturing, thereby negating its affect. Accordingly, there remains a need to provide methods for using electrochemical deposition techniques to provide discrete regions of CPP, including hydroxyapatite.

US 6,764,769 B2 discloses an apatite-coated metallic material, the coating of which consists of a covering of hydroxyapatite crystals and/or amorphous calcium phosphate spheres.

WO 98/13539 A1 discloses a method for coating a calcium phosphate compound onto a metallic material, the method comprising electrodepositing the calcium phosphate compound from an aqueous solution containing calcium ions, phosphate ions and a complex forming agent onto an electrode comprising the metallic material.

WO 2008/146113 A2 discloses a process for coating a surface of a metal element, the process comprising immersing into an electrolytic bath comprising collagen, calcium ions and phosphate ions a cathode and an anode, said cathode comprising the metal element to be coated.

US 5,310,464 discloses an electrolytic method for providing bone-emulating, phosphate coatings on prosthetic appliances. The appliance is thereby immersed in a phosphate-containing electrolyte to serve as the cathode of the electrolysis process.

DE 101 58 302 A1 discloses bioactive hydroxyapatite coatings on implants having metallic surfaces.

WO 98/09006 A1 discloses a method for electrochemical phosphating of metal surfaces by means of a cathodic process applying an aqueous phosphating solution.

US 2002/0084194 A1 discloses an article coated with an electrolytically deposited biocompatible composite layer useful as an internal prosthetic device. The coating comprises hydroxyapatite and chitosan.

### SUMMARY

The present technology provides methods for electrochemically depositing one or more discrete, discontinuous regions of a calcium phosphate onto a medical implant. The implant has at least one area having an electroconductive surface. At least a portion of the electroconductive surface is contacted with an electrolyte solution comprising calcium ions and phosphate ions. An electrical potential is applied between the electroconductive surface and the electrolyte solution. A plurality of discrete regions of a calcium phosphate phase is formed onto the electroconductive surface, wherein the calcium phosphate phase comprises a needle-shaped morphology.

In one embodiment, the present invention provides a method for electrochemically depositing discrete discontinuous regions of a calcium phosphate comprising hydroxyapatite onto a metallic surface of a medical implant comprising at least one area having an electroconductive surface, the electroconductive surface having at least one nano-scale textured region,
and wherein the electrochemical deposition is carried out in an electrolysis cell, or bath, in which at least the metallic surface of the implant is cathodically polarized,
the method comprising:
a. contacting at least a portion of the electroconductive surface of the implant with an electrolyte solution comprising calcium ions and phosphate ions having calcium ions at a concentration of about 1.7 mM and phosphate ions at a concentration of about 1.0 mM, wherein the pH of the electrolyte solution is maintained at 5-7 using hydrochloric acid or ammonium hydroxide; and
b. applying an electrical potential between the electroconductive surface and the electrolyte solution, wherein a current density of 40 mA/cm² is applied for 2 to 5 min, thereby forming a plurality of discrete discontinuous regions of the calcium phosphate onto the electroconductive surface, wherein the calcium phosphate comprises a needle-shaped morphology, and to the extent the implant includes nano-scale texturing, it is not covered by a complete coating of an amorphous calcium phosphate phase; and
c. subsequently rinsing or anodizing the implant.

In another embodiment the present invention provides a method for electrochemically depositing discrete discontinuous regions of a calcium phosphate comprising hydroxyapatite onto a metallic surface of a medical implant comprising at least one area having an electroconductive surface, the electroconductive surface having at least one nano-scale textured region,
and wherein the electrochemical deposition is carried out in an electrolysis cell, or bath, in which at least the metallic surface of the implant is cathodically polarized,
the method comprising:
a. contacting at least a portion of the electroconductive surface of the implant with an electrolyte solution, wherein the electrolyte solution has a pH of 6, a concentration of calcium ions of 0.2 mM and a concentration of phosphate ions of 0.1 mM; and
b. applying an electrical potential between the electroconductive surface and the electrolyte solution, wherein a current density of 30 mA/cm² is applied for 10 min at ambient temperature, thereby forming a plurality of discrete discontinuous regions of a calcium phosphate onto the electroconductive surface, wherein the calcium phosphate comprises a needle-shaped morphology, and to the extent the implant includes nano-scale texturing, it is not covered by a complete coating of an amorphous calcium phosphate phase; and
c. subsequently rinsing or anodizing the implant.

### DRAWINGS

Figure 1 is a SEM micrograph magnified about 80,000x illustrating discrete regions of hydroxyapatite deposited on a titanium substrate and having a needle-like morphology; and
Figures 2 and 3 are SEM micrographs magnified about 10,000x illustrating discrete regions of hydroxyapatite deposited on a titanium substrate having a needle-like morphology.

It should be noted that the figures set forth herein are intended to exemplify the general characteristics of materials, methods and devices among those of the present technology, for the purpose of the description of certain embodiments. These figures may not precisely reflect the characteristics of any given embodiment, and are not necessarily intended to define or limit specific embodiments within the scope of this technology.

### DETAILED DESCRIPTION

The following description of technology is merely exemplary in nature of the subject matter, manufacture and use of one or more inventions, and is not intended to limit the scope, application, or uses of any specific invention claimed in this application or in such other applications as may be filed claiming priority to this application, or patents issuing therefrom.

The headings (such as "Introduction" and "Summary") and subheadings used herein are intended only for general organization of topics within the present disclosure, and are not intended to limit the disclosure of the technology or any aspect thereof. In particular, subject matter disclosed in the "Introduction" may include novel technology and may not constitute a recitation of prior art. Subject matter disclosed in the "Summary" is not an exhaustive or complete disclosure of the entire scope of the technology or any embodiments thereof. Classification or discussion of a material within a section of this specification as having a particular utility is made for convenience, and no inference should be drawn that the material must necessarily or solely function in accordance with its classification herein when it is used in any given composition.

The description and specific examples, while indicating embodiments of the technology, are intended for purposes of illustration only and are not intended to limit the scope of the technology. Moreover, recitation of multiple embodiments having stated features is not intended to exclude other embodiments having additional features, or other embodiments incorporating different combinations of the stated features. Specific examples are provided for illustrative purposes of how to make and use the compositions and methods of this technology and, unless explicitly stated otherwise, are not intended to be a representation that given embodiments of this technology have, or have not, been made or tested.

As used herein, the words "desirable", "preferred" and "preferably" refer to embodiments of the technology that afford certain benefits, under certain circumstances. Furthermore, the recitation of one or more preferred or desired embodiments does not imply that other embodiments are not useful, and is not intended to exclude other embodiments from the scope of the technology.

As used herein, the word "include," and its variants, is intended to be non-limiting, such that recitation of items in a list is not to the exclusion of other like items that may also be useful in the materials, compositions, devices, and methods of this technology. Similarly, the terms "can" and "may" and their variants are intended to be non-limiting, such that recitation that an embodiment can or may comprise certain elements or features does not exclude other embodiments of the present technology that do not contain those elements or features.

Although the open-ended term "comprising," as a synonym of non-restrictive terms such as including, containing, or having, is used herein to describe and claim embodiments of the present technology, embodiments may alternatively be described using more limiting terms such as "consisting of' or "consisting essentially of." Thus, for any given embodiment reciting materials, components or process steps, the present technology also specifically includes embodiments consisting of, or consisting essentially of, such materials, components or processes excluding additional materials, components or processes (for consisting of) and excluding additional materials, components or processes affecting the significant properties of the embodiment (for consisting essentially of), even though such additional materials, components or processes are not explicitly recited in this application. For example, recitation of a composition or process reciting elements A, B and C specifically envisions embodiments consisting of, and consisting essentially of, A, B and C, excluding an element D that may be recited in the art, even though element D is not explicitly described as being excluded herein.

As referred to herein, all compositional percentages are by weight of the total composition, unless otherwise specified. Disclosures of ranges are, unless specified otherwise, inclusive of endpoints. Thus, for example, a range of "from A to B" or "from about A to about B" is inclusive of A and of B. Disclosure of values and ranges of values for specific parameters (such as temperatures, molecular weights, weight percentages, etc.) are not exclusive of other values and ranges of values useful herein.

When an element or layer is referred to as being "on", "engaged to", "connected to" or "coupled to" another element or layer, it may be directly on, engaged, connected or coupled to the other element or layer, or intervening elements or layers may be present. In contrast, when an element is referred to as being "directly on", "directly engaged to", "directly connected to" or "directly coupled to" another element or layer, there may be no intervening elements or layers present. Other words used to describe the relationship between elements should be interpreted in a like fashion (e.g., "between" versus "directly between," "adjacent" versus "directly adjacent," etc.). As used herein, the term "and/or" includes any and all combinations of one or more of the associated listed items.

The present technology provides methods for electrochemically depositing discrete, discontinuous regions of a calcium phosphate phase onto a medical implant. Titanium and its alloys, in addition to other metal substrates, are becoming increasingly popular as implant materials due to their favorable biocompatibility and favorable mechanical and chemical properties. At the same time, efforts continue to be made to improve bioinert behavior of implant materials. Calcium phosphate phases (CPP) have a lot of bioactive potential, thus enabling chemical bonding to natural bone. As used herein, the main inorganic constituent CPP may contain amorphous calcium phosphate (Ca₉(PO₄)₆ • nH₂O), hydroxyapatite (Ca₁₀(PO₄)₆(OH)₂), octacalcium phosphate (Ca₈H₂ (PO)₆H₂O), or brushite (CaHPO₄ • 2H₂O), or mixtures thereof. The CPP can additionally be doped with ions such as fluoride, silver, magnesium, carbonate, strontium, or sodium.

As is known in the art, hydroxyapatite (Ca₁₀(PO₄)₆(OH)₂) is a CPP biocompatible material that is similar in composition to the major inorganic mineral content of natural bone. As such, hydroxyapatite coatings provided on metallic or otherwise electroconductive medical implants can enhance an implant's osteoconductivity potential. Common deposition techniques for coating hydroxyapatite onto implants can include plasma spray coating, electrochemical deposition, and sol-gel deposition. While plasma spray coating is a widely used method, its high process conditions (high temperature) can result in coating properties that deviate from the mineral phase of bone, especially with respect to crystal structure and solubility. For example, the high process temperatures may cause partial decomposition of hydroxyapatite, resulting in the formation of other CPP, including amorphous calcium phosphate (ACP), α-tricalcium phosphate (TCP), β-TCP, tetracalcium phosphate, and calcium oxide. Numerous studies have found that more mechanical failure occurs at the metal/hydroxyapatite interface, rather than at the bone/hydroxyapatite interface. Accordingly, electrochemical deposition techniques are advantageous.

One problem with the known deposition techniques is the time required in order to obtain a crystalline hydroxyapatite structure, having needle-like morphology, from an amorphous precursor that is formed and subsequently changed into a crystalline material, mimicking *in vivo* mineralization process. Typically, spheres begin to grow at energetically favored places, commonly identified as the "ACP phase." The ACP is then transformed to the crystalline phase of hydroxyapatite. For example, small calcium phosphate precursor island regions are first formed that coalesce and form a continuous, homogeneous pre-layer on the metal surface. Both the pre-layer and the spheres comprise clusters of Ca₃(PO₄)₂ from which preferential crystalline hydroxyapatite needles grow:

Ca₃(PO₄)₂ + Ca²⁺ + 2 OH⁻ → Ca₁₀(PO₄)₆(OH)₂

While this two-phase process has many beneficial aspects, a more efficient means of hydroxyapatite deposition may include the direct deposition of hydroxyapatite crystalline onto a metal substrate, or a more timely transformation to the crystalline phase. Such a direct application can be beneficial where surfaces of the implant include nano-scale texturing or etching.

The present technology provides an electrochemical deposition process to facilitate an early transition from ACP to discrete deposition regions of hydroxyapatite crystalline, without the formation of a continuous layer of ACP as one would expect with such a deposition process. Unless one painstakingly masks various areas of the implant prior to the treatment, the typical electrochemical deposition process will first provide a continuous coating layer over the entire implant that is subsequently transformed into hydroxyapatite. Such a continuous coating would likely negate the various benefits obtained from any nano-scale etching or texturing. The present technology surprisingly provides the electrochemical deposition of discrete regions of CPP, and hydroxyapatite in particular, onto the surface of a medical implant. The present technology affects the kinetics of reaction, which can be controlled with the appropriate electrochemical parameters, as discussed below. In particular, in various embodiments, it provides a CPP deposition that is predominantly needle-shaped hydroxyapatite after only a short duration of time. For example, from about 70 to about 90 percent, or from about 85 to about 90 percent of the discrete CPP regions may have a crystalline structure, while only from about 10 to about 30 percent of the CPP may be an amorphous phase. This can provide for calcium phosphate regions of variable solubility. In certain embodiments, it may be preferred that the hydroxyapatite has a random orientation.

In the embodiments of the present technology, a medical implant is provided including at least one area having an electroconductive surface. The electroconductive surface can be a discrete area or it can be a continuous area covering the surface of the entire implant. The surface is provided with nano-scale texturing. Such an electroconductive surface can comprise a material selected from the group consisting of titanium, a titanium alloy, titanium nitrate, a CoCrMo alloy, stainless steel, an electroconductive polymer, and mixtures thereof.

The electrochemical deposition can be carried out in an electrolysis cell, or bath, in which at least the metallic surface of the implant is cathodically polarized. For example, a three-electrode arrangement can be made including a calomel electrode used as a reference electrode, a platinum sheet or gauze used as the counter electrode, and the metallic implant provided as the cathode. The deposition process can take place biomimetically, near physiological pH and temperature conditions.

At least a portion of the electroconductive surface is placed in contact with an electrolyte solution comprising calcium ions and phosphate ions. For example, the electrolyte can comprise a Ca²⁺/HₓPO₄^{(3-x)-} containing solution. The ratio of the concentration of the calcium ions and the phosphate ions is chosen such that it is equal or at least equivalent to their concentrations in hydroxyapatite. The electrolyte solution may include calcium chloride, calcium chloride dihydrate, or calcium acetate as the source of calcium ions, and ammonium dihydrogen phosphate as the source of phosphate ions. The choice of the particular salts used may be based on availability. The electrolyte solution is prepared using solutions that correspond to a final concentration of calcium:phosphate of about 1.7:1 (e.g., 1.67:1). In terms of actual concentration of the calcium and phosphate ions, one embodiment currently provides for a standard-like concentration of calcium ions of about 1.7 mM (e.g., 1.7 mM) and a concentration of phosphate ions of about 1.0 mM. Such a concentration calls for the electrical potential to be applied for 2 to 5 minutes, preferably about 2.5 minutes, in order to obtain desired deposition. In another embodiment, it is possible to decrease the concentration to about 1/10^{th}, or less, of the standard-like concentration. For example, the concentration of calcium ions may be provided at about 0.2 mM (e.g., 0.167 mM) while the phosphate ions are provided at about 0.1 mM. For embodiments having lower concentrations, an addition modification includes applying the electrical potential having a similar current density for a slightly longer period of time. With such a lower concentration of ions, the electrical potential isapplied for about 10 minutes, in order to obtain desired deposition. Even with the variance in the concentration levels, it is envisioned that the current density will still be applied at about the same level, or slightly lower, as will be discussed. It should be understood that the actual current density required may vary for each different type of component processed, and may depend upon the total surface area and surface finish, as well as the power sources available.

Once contact has been established between the electroconductive or metallic surface of the implant and the electrolyte solution, for example, by immersing the implant into an electrolyte bath, an electrical potential is applied between the electroconductive surface and the electrolyte solution. In one embodiment, the present technology provides applying an electrical potential having a constant current density of 40 mA/cm² for a period of time of 2 to 5 minutes. During this short period of time and at such an elevated current density, a high flux of ions rapidly moves toward the cathode and a plurality of discrete regions of a calcium phosphate phase are deposited on the electroconductive surface of the implant. Without limiting the mechanism, function or utility of the present technology, it is believed that, in embodiments having the appropriate concentration levels, heterogeneous nucleation or precipitation may occur within the solution near the implant surface that additionally settles on the implant surface. In another embodiment, the present technology provides applying an electrical potential having a constant current density of 30 mA/cm² for a period of time of 10 minutes.

Specifically, the present technology provides beginning with an electrolyte solution containing calcium and phosphate ions and leading to the predominant electrochemical deposition of highly desirable hydroxyapatite crystalline having needle-shaped morphology on the surface of an implant. The hydroxyapatite is deposited as homogeneous and discrete island type regions. Thus, to the extent the implant includes nano-scale texturing, it is not covered by a complete coating of an amorphous calcium phosphate phase, as it would be with conventional electrochemical deposition techniques. As described herein, the morphology of the hydroxyapatite crystals can be visually described as needle-like or needle-shaped, and in various embodiments having needles with dimensions of less than about 500 nm in length and less than about 60 nm in width, and in some embodiments less than about 30 nm in width. Typical needle lengths may be from about 200 and about 300 nm in certain embodiments, or from about 90 and about 140 nm in other embodiments. Depending upon the various parameters, it may be possible to obtain a slightly mixed state of hydroxyapatite and amorphous calcium phosphate phase, provided that the electrochemical deposition still provides homogeneous, discrete, discontinuous island-type coating regions.

Electrochemical deposition of a calcium phosphate phase depends in part on the pH-dependent solubility of the calcium phosphate, which has been found to decrease with increasing pH. Using an electrochemical deposition process, one can control the pH at the cathode/electrolyte interface. As is known in the art, during cathodic polarization of a metal in an aqueous electrolyte, the following reactions occur at the surface of the cathode (reduction of water, proton discharge, and reduction of dissolved oxygen):

2H₂O + 2e⁻ → H₂ + 2OH⁻

2H₃O⁺ + 2e⁻ → H₂ + 2H₂O

O₂ + H₃O⁺ + 4e⁻ → 3OH⁻

resulting in the formation of hydroxyl ions and hence alkalization close to the surface. In the case of a metal implant comprising titanium, the calcium and phosphate ions react with the hydroxyl groups on the titanium surface because of heterogeneous nucleation. Hydroxyl ions from the cathodic sub process (above) hydroxylate the titanium surface by physical and chemical adsorption:

TiO₂ + H₂O → TiO(OH)₂

Additionally, it is known that increased cathodic polarization is associated with increased hydrogen production and oxygen depletion of the titanium surface because of the partial reduction of titanium dioxide:

TiO₂ + 2H₂O + e⁻ → Ti(OH)₃ + OH⁻

Thus in one embodiment, the pH of the electrolyte solution is maintained at from about 5 to about 7, using hydrochloric acid or ammonium hydroxide. For some applications, it may be desirable to maintain the pH at the near physiological condition of about 6 (e.g., about 6.4). In certain other embodiments, because of the desire to avoid a continuous coating of CPP on the metal implant, the electrolyte solution can be maintained slightly acidic, for example, at a level of from about 5 to about 6. This slightly acidic environment allows for the partial dissolution of the CPP to occur in equilibrium with the precipitation and deposition processes.

While it is believed that the CPP deposition process is accelerated with increasing current density, the formation of CPP on a metal surface is generally controlled by a nucleation mechanism as the initial growth step. With increasing current density, however, hydrogen gas development is also increased. Accordingly, care must be taken into consideration because hydrogen bubbles may initiate a faster electrolyte exchange in front of the cathode and increase the diffusion of the electrolyte ions due to a thinner diffusion boundary layer. Excessive hydrogen bubbling may also interfere with the electrochemical deposition process and prevent homogeneous CPP formation. Accordingly, in various embodiments, the present technology provides placing the implants in a bath containing the electrolyte solution and rotating the implants during application of the electrical potential.

The present technology also provides for larger scale processes for making a plurality of medical implants having discrete regions of a calcium phosphate phase deposited thereon. It is envisioned that the process can treat from 2 up to 70 or more implants at one time, depending upon the size and surface area of the implants, as well as the desired electrochemical deposition parameters, including the available power supply.

The process can include preparing an electrolyte solution comprising calcium ions and phosphate ions having a concentration ratio of calcium:phosphate of about 1.7:1 as previously described. A plurality of implants is then placed into the electrolyte solution, or bath. Any debris on the implant surface may lead to uncoated areas. Accordingly, the implants can optionally be cleaned prior to the deposition process, for example using an appropriate ultrasonic type wash. In certain embodiments, the electrolyte solution is provided in an inner bath container that is placed or disposed within an appropriate outer bath container. The outer bath container can be provided with circulating water to maintain a consistent temperature of the inner bath, for example, at about ambient temperature or alternatively about 37°C. Each implant comprises at least one area having an electroconductive surface which, in various embodiments, includes a metallic area or surface. These electroconductive surfaces are appropriately connected and used as the cathodes for cathodic polarization. A constant electrical potential is applied between the cathodes and the electrolyte solution, wherein the electrical potential has a constant current density of 40 mA/cm². As previously discussed, the electrical potential can be applied for a period of time of 2 to 5 minutes depending on the remaining deposition parameters and desired amount of hydroxyapatite deposition. In another embodiment, a current density of 30 mA/cm² is applied for 10 minutes. The process includes electrochemically depositing a plurality of discrete regions of needle-shaped hydroxyapatite crystals onto the electroconductive surfaces. The implants can be appropriately rotated during the application of electrical potential, depending on the amount of hydrogen bubbling that may occur. In various aspects, once the electrochemical deposition is complete, the implants can be removed and sent to a rinsing station. Depending on the particular metal used, the implants can also be sent to an appropriate anodizing station. Such an anodizing bath may be provided including deionized water, trisodium phosphate dodecahydrate, and di-potasium hydrogen phosphate at ambient temperature.

In certain embodiments, the electrochemical deposition process may be carried out by cathodic polarization in a number of successive, repeated process cycles. For example, a process cycle may include cathodic polarization in one or more successive steps, in certain embodiments during at least two discrete intervals of time, with identical or different (increased or decreased) constant current densities, and a rinsing and/or drying phase following thereon.

The present technology is further illustrated through the following non-limiting examples.

### Example 1

A disc of Ti6A14V having a radius of about 0.5 inches and a thickness of 0.25 inches is prepared with a smooth machine finish, cleaned in an ultrasonic bath, and rinsed with distilled water. The thickness portion is masked and the disc sample is placed into an electrolyte solution at ambient temperature including 150 ml each of a stock solution of CaCl₂ and NH₄H₂PO₄ in concentrations of 33 mM and 20 mM, respectively. Deionized water is added providing a 3 L total volume solution having a final concentration of 1.67 mM calcium ions and 1.0 mM phosphate ions. The pH is adjusted to 5.1 using hydrochloric acid.

After connection to a potentiostat, electrochemical deposition is carried out by means of galvanostatic polarization under cathodic current flow at a current density of about 40 mA/cm² in order to provide a high flux of ions toward the cathode. After a deposition time of about 2.5 minutes, the cathodic polarization is complete and the sample is removed and rinsed with deionized water. Electron microscopic examination reveals a plurality of discrete but homogenous regions of CPP having needle like morphology as shown in Figure 1. Further IR-spectroscopic investigations provide proof that the discrete crystalline mineral phase comprises hydroxyapatite.

### Example 2 (Comparative)

A disc of Ti6A14V is prepared as in Example 1. The disc sample is placed into an electrolyte solution at ambient temperature including 15 ml each of a stock solution of CaCl₂ and NH₄H₂PO₄ in concentrations of 33 mM and 20 mM, respectively. Deionized water is added providing a 3 L total volume solution having a final concentration of 0.167 mM calcium ions and 0.1 mM phosphate ions. The pH is adjusted to 6.4 using ammonium hydroxide.

After connection to a potentiostat, electrochemical deposition is carried out by means of galvanostatic polarization under cathodic current flow at a current density of about 20mA/cm² in order to provide a high flux of ions toward the cathode. After a deposition time of about 10 minutes, the cathodic polarization is complete and the sample is removed and rinsed with deionized water. Electron microscopic examination reveals a plurality of discrete but homogenous regions of CPP having needle like morphology as shown in Figure 2. Further IR-spectroscopic and X-ray diffraction investigations provide proof that the discrete crystalline mineral phase comprises hydroxyapatite.

### Example 3

A disc of Ti6A14V is prepared as in Example 1. The disc sample is placed into an electrolyte solution at ambient temperature including 15 ml each of a stock solution of CaCl₂ and NH₄H₂PO₄ in concentrations of 33 mM and 20 mM, respectively. Deionized water is added providing a 3 L total volume solution having a final concentration of 0.167 mM calcium ions and 0.1 mM phosphate ions. The pH is adjusted to 6.4 using ammonium hydroxide.

After connection to a potentiostat, electrochemical deposition is carried out by means of galvanostatic polarization under cathodic current flow at a current density of about 30mA/cm² in order to provide a high flux of ions toward the cathode. After a deposition time of about 10 minutes, the cathodic polarization is complete and the sample is removed and rinsed with deionized water. Electron microscopic examination reveals a plurality of discrete but homogenous regions of CPP having needle like morphology as shown in Figure 3. Further IR-spectroscopic and X-ray diffraction investigations provide proof that the discrete crystalline mineral phase comprises hydroxyapatite.

The embodiments described herein are exemplary and not intended to be limiting in describing the full scope of compositions and methods of the present technology. Equivalent changes, modifications and variations of embodiments, materials, compositions and methods can be made within the scope of the present technology, as defined in the appended claims, with substantially similar results.

## Claims

1. A method for electrochemically depositing discrete discontinuous regions of a calcium phosphate comprising hydroxyapatite onto a metallic surface of a medical implant comprising at least one area having an electroconductive surface, the electroconductive surface having at least one nano-scale textured region,
and wherein the electrochemical deposition is carried out in an electrolysis cell, or bath, in which at least the metallic surface of the implant, is cathodically polarized,
the method comprising:
a. contacting at least a portion of the electroconductive surface of the implant with an electrolyte solution comprising calcium ions and phosphate ions having calcium ions at a concentration of 1.7 mM and phosphate ions at a concentration of 1.0 mM, wherein the pH of the electrolyte solution is maintained at 5-7 using hydrochloric acid or ammonium hydroxide; and
b. applying an electrical potential between the electroconductive surface and the electrolyte solution, wherein a current density of 40 mA/cm² is applied for 2 to 5 min, thereby forming a plurality of discrete discontinuous regions of the calcium phosphate onto the electroconductive surface, wherein the calcium phosphate comprises a needle-shaped morphology, and to the extent the implant includes nano-scale texturing, it is not covered by a complete coating of an amorphous calcium phosphate phase; and
c. subsequently rinsing or anodizing the implant.

2. A method for electrochemically depositing discrete discontinuous regions of a calcium phosphate comprising hydroxyapatite onto a metallic surface of a medical implant comprising at least one area having an electroconductive surface, the electroconductive surface having at least one nano-scale textured region,
and wherein the electrochemical deposition is carried out in an electrolysis cell, or bath, in which at least the metallic surface of the implant, is cathodically polarized,
the method comprising:
a. contacting at least a portion of the electroconductive surface of the implant with an electrolyte solution, wherein the electrolyte solution has a pH of 6, a concentration of calcium ions of 0.167 mM and a concentration of phosphate ions of 0.1 mM; and
b. applying an electrical potential between the electroconductive surface and the electrolyte solution, wherein a current density of 30 mA/cm² is applied for 10 min at ambient temperature, thereby forming a plurality of discrete discontinuous regions of the calcium phosphate onto the electroconductive surface, wherein the calcium phosphate comprises a needle-shaped morphology, and to the extent the implant includes nano-scale texturing, it is not covered by a complete coating of an amorphous calcium phosphate phase; and
c. subsequently rinsing or anodizing the implant.

## Patentansprüche

1. Verfahren zum elektrochemischen Abscheiden diskreter, diskontinuierlicher Bereiche eines Hydroxyapatit enthaltenden Calciumphosphats auf eine metallische Oberfläche eines medizinischen Implantats, das zumindest ein Gebiet mit einer elektrisch leitfähigen Oberfläche umfasst, wobei die elektrisch leitfähige Oberfläche zumindest einen im Nanomaßstab strukturierten Bereich aufweist,
und wobei das elektrochemische Abscheiden in einer Elektrolysezelle oder einem Bad durchgeführt wird, worin zumindest die metallische Oberfläche des Implantats kathodisch polarisiert ist,
wobei das Verfahren umfasst:
a. in Kontakt Bringen zumindest eines Teils der elektrisch leitfähigen Oberfläche des Implantats mit einer Elektrolytlösung, die Calciumionen und Phosphationen enthält und eine Konzentration an Calciumionen von 1,7 mM und eine Konzentration an Phosphationen von 1,0 mM aufweist, wobei der pH-Wert der Elektrolytlösung mittels Salzsäure oder Ammoniumhydroxid bei 5-7 gehalten wird; und
b. Anlegen eines elektrischen Potentials zwischen der elektrisch leitfähigen Oberfläche und der Elektrolytlösung, wobei für 2 bis 5 Minuten eine Stromdichte von 40 mA/cm² angelegt wird, wodurch eine Mehrzahl diskreter, diskontinuierlicher Bereiche des Calciumphosphats auf der elektrisch leitfähigen Oberfläche gebildet wird, wobei das Calciumphosphat eine nadelförmige Morphologie umfasst, und wobei das Implantat in dem Ausmaß, in dem es eine Strukturierung im Nanomaßstab aufweist, nicht von einer vollständigen Beschichtung aus einer amorphen Calciumphosphat-Phase bedeckt wird; und
c. anschließendes Spülen oder Anodisieren des Implantats.

2. Verfahren zum elektrochemischen Abscheiden diskreter, diskontinuierlicher Bereiche eines Hydroxyapatit enthaltenden Calciumphosphats auf eine metallische Oberfläche eines medizinischen Implantats, das zumindest ein Gebiet mit einer elektrisch leitfähigen Oberfläche umfasst, wobei die elektrisch leitfähige Oberfläche zumindest einen im Nanomaßstab strukturierten Bereich aufweist,
und wobei das elektrochemische Abscheiden in einer Elektrolysezelle oder einem Bad durchgeführt wird, worin zumindest die metallische Oberfläche des Implantats kathodisch polarisiert ist,
wobei das Verfahren umfasst:
a. in Kontakt Bringen zumindest eines Teils der elektrisch leitfähigen Oberfläche des Implantats mit einer Elektrolytlösung, wobei die Elektrolytlösung einen pH-Wert von 6, eine Calciumionen-Konzentration von 0,167 mM und eine Phosphationen-Konzentration von 0,1 mM aufweist; und
b. Anlegen eines elektrischen Potentials zwischen der elektrisch leitfähigen Oberfläche und der Elektrolytlösung, wobei für 10 Minuten bei Raumtemperatur eine Stromdichte von 30 mA/cm² angelegt wird, wodurch eine Mehrzahl diskreter, diskontinuierlicher Bereiche des Calciumphosphats auf der elektrisch leitfähigen Oberfläche gebildet wird, wobei das Calciumphosphat eine nadelförmige Morphologie umfasst, und wobei das Implantat in dem Ausmaß, in dem es eine Strukturierung im Nanomaßstab aufweist, nicht von einer vollständigen Beschichtung aus einer amorphen Calciumphosphat-Phase bedeckt wird; und
c. anschließendes Spülen oder Anodisieren des Implantats.

## Revendications

1. Procédé de dépôt électrochimique de régions discontinues discrètes d'un phosphate de calcium comprenant de l'hydroxyapatite sur une surface métallique d'un implant médical comprenant au moins une zone ayant une surface électroconductrice, la surface électroconductrice présentant au moins une région texturée à l'échelle nanoscopique,
et dans lequel le dépôt électrochimique est effectué dans une cellule ou un bain d'électrolyse, dans laquelle ou lequel au moins la surface métallique de l'implant est polarisée cathodiquement,
le procédé comprenant les étapes consistant à :
a. mettre en contact au moins une partie de la surface électroconductrice de l'implant avec une solution électrolytique comprenant des ions calcium et des ions phosphate ayant des ions calcium à une concentration de 1,7 mM et des ions phosphate à une concentration de 1,0 mM, le pH de la solution électrolytique étant maintenu à 5-7 en utilisant de l'acide chlorhydrique ou de l'hydroxyde d'ammonium ; et
b. appliquer un potentiel électrique entre la surface électroconductrice et la solution électrolytique, une densité de courant de 40 mA/cm² étant appliquée pendant 2 à 5 min, formant ainsi une pluralité de régions discontinues discrètes du phosphate de calcium sur la surface électroconductrice, le phosphate de calcium comprenant une morphologie en aiguilles, et dans la mesure où l'implant inclut une texturation à échelle nanoscopique, il n'est pas couvert par une couche complète d'une phase de phosphate de calcium amorphe ; et
c. rincer ou anodiser ensuite l'implant.

2. Procédé de dépôt électrochimique de régions discontinues discrètes d'un phosphate de calcium comprenant de l'hydroxyapatite sur une surface métallique d'un implant médical comprenant au moins une zone ayant une surface électroconductrice, la surface électroconductrice présentant au moins une région texturée à l'échelle nanoscopique,
et dans lequel le dépôt électrochimique est effectué dans une cellule ou un bain d'électrolyse, dans laquelle ou lequel au moins la surface métallique de l'implant est polarisée cathodiquement,
le procédé comprenant les étapes consistant à :
a. mettre en contact au moins une partie de la surface électroconductrice de l'implant avec une solution électrolytique, la solution électrolytique ayant un pH de 6, une concentration en ions calcium de 0,167 mM et une concentration en ions phosphate de 0,1 mM ; et
b. appliquer un potentiel électrique entre la surface électroconductrice et la solution électrolytique, une densité de courant de 30 mA/cm² étant appliquée pendant 10 min à température ambiante, formant ainsi une pluralité de régions discontinues discrètes du phosphate de calcium sur la surface électroconductrice, le phosphate de calcium comprenant une morphologie en aiguilles, et dans la mesure où l'implant inclut une texturation à échelle nanoscopique, il n'est pas couvert par une couche complète d'une phase de phosphate de calcium amorphe ; et
c. rincer ou anodiser ensuite l'implant.
